

# UNITED STATES PATENT OFFICE.

THOMAS C. JAMES, OF CHICAGO, ILLINOIS.

## SOLUTION FOR WATERPROOFING FABRICS.

Specification of Letters Patent. Patented Sept. 18, 1917.

1,240,345.

No Drawing.

Application filed September 30, 1914. Serial No. 364,223.

To all whom it may concern:

Be it known that I, THOMAS C. JAMES, a citizen of the United States, and a resident of Chicago, in the county of Cook and State of Illinois, have invented certain new and useful Improvements in Solutions for Waterproofing Fabrics; and I do hereby declare that the following is a full, clear, and exact description thereof.

10 This invention relates to an improved solution for water-proofing fabrics and consists of the matters hereinafter described and more particularly pointed out in the appended claim.

15 The object of my invention is to produce a mixture or preparation for the purpose of water proofing fabrics, superior to the preparations now in use, which may be prepared with ease and at considerable less cost than 20 the cost of preparations now used for similar purposes.

In carrying out my formula I make a mixture of one-half pound of acetate of lead and one-half pound of powdered alum, with 25 three gallons of water, and place the same in a suitable vessel. This mixture is agitated or stirred until the acetate of lead and the alum is thoroughly dissolved therein, after which the solution is left at rest for 30 a suitable length of time, to permit of the deposit of sediment on the bottom of the vessel. The solution or mixture in the vessel is then withdrawn by means of a siphon or any suitable device which will not dis- 35 turb the sediment in said vessel, and is then measured and placed in a second vessel provided therefor.

For each gallon of the drawn off mixture and in proportionate amounts for each 40 proportionate part of a gallon, I add one ounce of gum arabic which has been dissolved in benzine or a similar hydrocarbon or in an alcoholic body such as wood alcohol. The gum arabic may be dissolved in 45 any other volatile chemical which is not in itself oleaginous or greasy.

To each one gallon of the solution of gum arabic, powdered alum and acetate of lead, and in a proportionate amount for each proportionate part of a gallon of said solution, I add two ounces of essential oil for the purpose of deodorizing or sweetening 50 of the mixture.

The water-proofing solution is now ready

for use and the manner of applying it to 55 the fabric for the purpose of making the latter impervious to water is as follows: Assuming the fabric to be in the bolt, said bolt is immersed in the solution and when thoroughly saturated or impregnated, the 60 bolt of fabric is removed from the solution and passed through a suitable compressing or wringing device to expel all the surplus solution therefrom. Thereafter the fabric may be dried by artificial means or by exposure to the atmosphere.

The solution may be applied equally as well to a ready made garment as to fabric in the bolt. In the case of a coat, uniform or the like, for example, the garment is 70 laid out flat upon a table or other suitable surface, and then saturated with the solution by a sponge or rag which has been dipped into the solution, or by other suitable means, by moving the wet sponge or 75 rag over the garment in the manner in which a tailor would dampen a garment for reason of pressing the same. After the garment has been thus treated with the water proofing solution, the garment may 80 be hung up to dry either in a drying room or in the atmosphere.

Fabrics after having been water-proofed with my improved solution, retain their original color and shape and the presence of 85 the water-proofing solution is not noticeable in the fabric even upon close inspection of the same. Any fabric, whether woven or knitted, regardless of its texture, may be so treated to make the same water proof. 90 Garments, after being treated with my improved solution may be worn without any discomfort to the wearer, so thoroughly does the solution impregnate the texture, and make the same thoroughly water-proof. 95 Exposure to the rain for hours will not change the fabric, so efficiently will the water-proofing shed the rain and moisture. It is also to be noted that my improved solution is not only highly efficient in use but 100 possesses other very desirable elements of utility, namely cheapness and simplicity in its preparation and in its application to fabrics.

Garments which have been treated with 105 my improved water-proofing solution beside possessing the advantages above mentioned, are rendered practically inflammable

and may also be pressed in the manner of ordinary garments without impairing its water or rain resisting qualities.

What I claim is:

- 5 A solution for water-proofing fabrics produced by dissolving like parts by weight of acetate of lead and of powdered alum in substantially twenty-five times their combined weight of water and mixing with this
- 10 solution substantially three-sixteenths of the combined weight of the lead acetate and

alum of gum arabic dissolved in an alcoholic body.

In testimony, that I, claim the foregoing as my invention I affix my signature in the 15 presence of two witnesses, this 26th day of September, A. D. 1914.

THOMAS C. JAMES.

Witnesses:

T. H. ALFREDS,  
KARL W. DOLL.